

Dec. 26, 1922.

1,439,907.

W. C. MAIN.

TREATMENT OF CAST IRON PARTICLES AND ARTICLES MADE THEREFROM.

FILED NOV. 17, 1920.



Fig. 1



Fig. 2



Fig. 3



Fig. 4

Inventor  
Walter C. Main  
By Day, Oberlin & Day  
Attorneys

## UNITED STATES PATENT OFFICE.

WALTER C. MAIN, OF LAKewood, OHIO.

## TREATMENT OF CAST-IRON PARTICLES AND ARTICLES MADE THEREFROM.

Application filed November 17, 1920. Serial No. 424,628.

*To all whom it may concern:*

Be it known that I, WALTER C. MAIN, a citizen of the United States, and a resident of Lakewood, county of Cuyahoga, and State of Ohio, have invented a new and useful Improvement in the Treatment of Cast-Iron Particles and Articles Made Therefrom, of which the following is a specification, the principle of the invention being 5 herein explained and the best mode in which I have contemplated applying that principle, so as to distinguish it from other inventions.

The invention herein relates to articles formed from cast iron particles and the treatment thereof before or after their formation into briquettes or other articles so that the finished product will retain its shape. This treatment is particularly useful in connection with briquettes used as 10 material for furnace charging and has in view the production of an article which may withstand the frequent handling necessary in such use, without fracturing or being reduced to powder through abrasive action 15 during shipment or transfer.

I have found that when briquettes are made of steel particles such as borings, turnings and the like, or of such particles of other metals, such as brass, copper and the 20 like, no difficulty is experienced in forming the same into briquettes which will successfully withstand hard usage. However, when particles of this character of cast iron are used for the briquette material, it is 25 found that they readily fracture, and cannot be handled or shipped without the greatest care.

The object of my invention is to so treat the material out of which briquettes are 30 formed or the briquettes themselves after being formed of cast iron particles as to make the finished briquettes of an extremely durable character, and equal for the purpose 35 in view to the briquettes manufactured of the other materials mentioned.

While I have particularly mentioned briquettes I do not mean to limit the application of my invention to any desired form of the finished article, whether in the shape 40 of rods, balls or any irregular form determined upon. To the accomplishment of the foregoing and related ends, said invention, then, consists of the method hereinafter

fully described and particularly pointed out in the claims.

The annexed drawing and the following description set forth in detail one method and one product exemplifying my invention, such disclosed procedure and product constituting, however, but one of various applications of the principles of my invention.

In said annexed drawing:—

Fig. 1 is a perspective view of a briquette of cylindrical shape to be treated by my method; Fig. 2 is a cross-section of a briquette, showing the change in the superficial character thereof produced through the use of my method of treatment; Fig. 3 is a perspective view of a form of briquette to which my treatment is particularly applicable, the ends of said briquette having dome-shaped portions of low elevation; and Fig. 4 is a cross-sectional view of the form illustrated in Fig. 3, showing the greater density of the outer portions of said briquette, and the results of the application of my treatment to this highly compacted surface.

After the briquettes are formed in the compressing apparatus of any preferred design, I subject them for a period of approximately five minutes to a bath of hydrochloric acid preferably of a strength of from three to five per cent. This I find produces a very tenacious superficial coating upon the briquette, which enables it to withstand any amount of handling in ordinary course of industry. Instead of treating the briquette after its formation in a press, I may treat the borings or other particles for a like period immediately prior to their compression. A difference is noted in the cohesive characteristics of the briquettes treated in each of these two manners, a greater degree of tenacity being exhibited by the briquettes formed of borings which receive preliminary treatment.

The following data is set down to show more particularly the character of the change produced:—

Physical tests.

Straight compression:

|                   |       |      |        |
|-------------------|-------|------|--------|
| As formed         | 14000 | lbs. | 100    |
| Treated briquette | 16000 | "    | 6 hrs. |
|                   | 17500 | "    | 24 "   |
| Treated borings   | 16080 | "    | 6 "    |
|                   | 18000 | "    | 24 "   |

|                                  |        |        |  |
|----------------------------------|--------|--------|--|
| Drop test (15 feet on concrete). |        |        |  |
| As formed                        | 1 fall |        |  |
| Treated briquette                | 4 "    | 6 hrs. |  |
|                                  | 8 "    | 24 "   |  |
| 5 Treated borings                | 5 "    | 6 "    |  |
|                                  | 12 "   | 24 "   |  |

## Analysis shows:

## Sulphur content—

|                   |      |
|-------------------|------|
| 10 Borings        | 124  |
| Treated briquette | 120  |
| Treated borings   | 116  |
| Percent oxide—    |      |
| Treated briquette | .020 |
| Treated borings   | .035 |

15 It will be noted that the treated briquette, whether such treatment is of the finished briquette or of the borings, exhibits a considerably greater resistance to compression than the briquette not so treated. This power of resistance increases after an interval of about twenty-four hours. By means of the drop test it will be noted, the treated briquette is four times as tenacious 25 as the ordinary briquette after a period of six hours has elapsed, and eight times as tenacious after twenty-four hours has elapsed. The treated borings more than double the resisting power of the briquette 30 after the lapse of twenty-four hours from that exhibited after a period of six hours. The treatment is also of advantage in reducing the sulphur content of the briquettes, the preliminary treatment of the borings 35 in this respect showing a less amount of sulphur than the briquettes treated after compression, but a greater percentage of oxide than the briquettes so treated.

40 I also find that the use of hydrochloric acid of the strength indicated produces a very rapid change in the material and no unfavorable incidental effects are noted such as secondary reactions or hygroscopic phenomena. The acid acts at once to produce 45 the cohesive coating to a certain degree and with a shallow depth of penetration. Substantially the maximum degree of tenacity is attained after the elapsing of the twenty-four hour period, but where the borings or 50 particles are treated prior to compression, such treatment must be immediately followed by the molding and compressing operation to insure the most effective results.

55 As a further development of my invention, I may combine the steps above outlined and after compressing a briquette from the treated borings give a further treatment to the finished briquette with hydrochloric acid of the strength indicated for 60 a slightly longer period or use acid of a slightly greater concentration, thus producing an outside area of greater depth of penetration than would be furnished by the acid

applied directly to the particles and insure a uniform coating of oxide upon the outside 65 surface of the briquette.

Other steps or forms may be employed embodying the features of my invention instead of the ones herein explained, change being made in the steps or forms, provided 70 those stated by any of the following claims or the equivalent thereof be employed.

I therefore particularly point out and distinctly claim as my invention:

1. A briquette formed of cast iron particles having an iron oxide exterior coating of uniform distribution, and highly cohesive character, and of merely superficial penetration, produced by treatment with hydrochloric acid. 75

2. A briquette of cast iron particles having a compressed central portion and a more highly compressed portion adjacent its surface, the last named portion having a superficial coating of small penetration to give to 80 the briquette a cohesive tenacious exterior to permit handling and shipping.

3. The method of producing a non-frangible article of cast iron particles which comprises treating such particles with hydrochloric acid to rapidly oxidize the same to make them cohesive when formed into finished products. 90

4. An article of compressed cast iron particles having a homogeneous central portion of medium compressed character, an exterior portion of substantial depth of highly compressed character, and a superficial portion of lesser depth than the last mentioned portion of a highly cohesive 100 character and modified form of the original substance. 95

5. The method of preparing cast iron particles for manufacture into non-frangible briquettes, which comprises the treatment 105 of such particles with hydrochloric acid and thereafter immediately compressing the same.

6. The method of preparing cast iron particles for use in a molding and compressing apparatus, which consists in subjecting said particles for a limited time to the action of hydrochloric acid to accelerate oxidation thereof, substantially as described. 110

7. The method of preparing cast iron particles for manufacture into non-frangible briquettes, which comprises the treatment of such particles with hydrochloric acid, thereafter immediately compressing the 120 same, and then subjecting the finished briquette to a slightly greater degree of action by such acid. 115

Signed by me, this 12th day of November, 1920.

WALTER C. MAIN.